

(No Model.)

H. HEINKE.

INK BLOTTER.

No. 379,067.

Patented Mar. 6, 1888.



Witnesses:

Alfred Jonghman.  
William Partington.

Inventor:

H. Heinke.  
by his attorneys,  
Roeder & Neisen.

# UNITED STATES PATENT OFFICE.

HORST HEINKE, OF NEW YORK, N. Y.

## INK-BLOTTER.

SPECIFICATION forming part of Letters Patent No. 379,067, dated March 6, 1888.

Application filed December 12, 1887. Serial No. 257,647. (No model.)

*To all whom it may concern:*

Be it known that I, HORST HEINKE, of New York city, New York, have invented a new and Improved Ink-Blotter, of which the following is a specification

5 This invention relates to a composition to be applied to a blotting-pad, and which will readily absorb the ink.

The invention consists in the various features of improvement, more fully pointed out in the claims.

The accompanying drawing represents a transverse section of a blotter containing my improvement.

15 The letter *a* represents a wooden block having handle *b* and provided with a sheet of felt, *c*, secured to its curved lower side. This sheet of felt *c* is coated with my improved compound, *d*, which is obtained as follows:

20 One pound of glue is boiled in ten quarts of water until the glue is dissolved. Then five pounds of chalk, one pound of powdered brick, and one-fourth pound of borax are added. The whole is thoroughly stirred and is applied to

25 the felt *c* by means of a brush. The coating thus applied will last for about a week, and may then be renewed with a brush, the mixture being well shaken before being reapplied.

An advantage of this composition lies in the fact that it permits ready renewal in a simple manner, and that thus the blotter will not become saturated, so as to become useless, as is the case with blotters and blotting compositions ordinarily employed.

The chalk in the composition serves as an absorbent. The powdered brick is also an absorbent, and at the same time constitutes the coloring-matter. The borax prevents discoloration—that is, it prevents the composition from coloring the paper—while the glue binds the materials and renders the mixture elastic when dry.

What I claim is—

1. A blotting composition consisting of glue, powdered brick, chalk, and borax, in about the proportions named, substantially as specified.

2. The combination of block *a* and felt *c* with a coating, *d*, consisting of glue, powdered brick, chalk, and borax, substantially as specified.

HORST HEINKE.

Witnesses:

HENRY E. ROEDER,  
F. V. BRLESEN.